

Nov. 30, 1937.

W. J. KOENIG

2,100,484

COMPOSITION AND DRYING OF THE SAME

Filed Feb. 23, 1935

2 Sheets-Sheet 1

FIG.-1



FIG.-2



INVENTOR

WALTER J. KOENIG

BY *Harry A. Mitten*  
ATTORNEY

Nov. 30, 1937.

W. J. KOENIG

2,100,484

COMPOSITION AND DRYING OF THE SAME

Filed Feb. 23, 1935

2 Sheets-Sheet 2

FIG.-3



INVENTOR  
WALTER J. KOENIG

BY  
Harry A. Midman  
ATTORNEY

## UNITED STATES PATENT OFFICE

2,100,484

## COMPOSITION AND DRYING OF THE SAME

Walter J. Koenig, Trenton, N. J., assignor to  
 Sloane-Blabon Corporation, Trenton, N. J., a  
 corporation of Delaware

Application February 23, 1935, Serial No. 7,717

7 Claims. (Cl. 91—70)

This invention relates to a drying oil composition and to method of drying oils. More particularly the invention relates to a composition and method in which surface distortion is prevented by protecting the surface of the oil against excessively rapid oxidation and especially by evaporating a non-oxidizing slowly volatile substance from said surface.

Certain oils, and especially China-wood oil, which possess extremely valuable properties in other respects, are subject to the great disadvantage that on drying tend to surface distortion thereby producing wrinkled and/or orange peel effects. These features are undesirable particularly when a smooth surface is desired, as, for example, in printed materials in the linoleum and felt base industry, or in any place where enamels, paints, varnishes, etc., using drying oils herein-after discussed, are used on a surface.

An additional disadvantage of the above described oils is the tendency of these oils to "skin" over or to harden while awaiting use.

It is, therefore, an object of my present invention to prevent or substantially reduce the tendency of such oils from wrinkling and/or orange peeling during the drying of the oils. An additional object is to substantially reduce the skinning-over tendency of paints or similar coating compositions in which such oils are used as vehicles.

I have found, through the medium of my invention hereinafter described, that surface distortion can be prevented or controlled and that even with very rapid drying at superatmospheric temperatures, smooth and substantially perfect films can be obtained if the surface of the film is protected from excessively rapid oxidation during the drying action. It is necessary that the drying proceed substantially uniformly throughout the film while the surface of the film is protected from oxidation through the medium of a protective non-oxidizing gaseous blanket at the interface of the surface to be dried and the atmosphere.

The protective blanket may be formulated in various ways, for example, by reducing the amount of oxygen in the atmosphere adjacent to the surface of the oil. This may be done, for example, by placing the film to be dried in a closed chamber and then replacing the air present therein with a non-oxidizing gas. The expense involved in making this method practical from a commercial viewpoint, and also the difficulties involved in controlling the non-oxidizing atmosphere, cause this method to be undesirable.

able. It is understood, however, that smooth films can be obtained by this method.

Due to the difficulties involved in the method described, I have found that it is more desirable to control the atmosphere immediately above the surface of the drying oil film by incorporating the protective substance in the film itself. If, for example, a non-oxidizing evaporating material is incorporated in the oil composition film to be dried, so that its vapors are given off from the surface during the drying period at super-atmospheric temperatures, a practical protection is secured and smooth films, either glossy or matte finishes, are readily obtained. It is, of course, desirable to avoid rapid circulation of the gases; the gases in the chamber should be substantially stagnant.

The protective agents or substances which are incorporated directly with the drying oil may be either reactive or non-reactive with the oil. I have found that in order to reduce costs in production, and at the same time reduce complications in the process, it is preferable to use substances which will condense with the drying oil and the uncondensed excess portion, on being volatilized, will form the protective layer above the film to be dried.

In considering reactive substances which will condense with the drying oil, as described in my co-pending application No. 646,148, filed December 7, 1932, of which the present application is a continuation in part, the condensing agent is supplied in excess and the uncondensed portion on volatilizing, preferably at super-atmospheric temperatures, will form the desired protective blanket. For example, in the preferred examples of application No. 646,148, the cyclohexanol and cyclohexanone were supplied in excess, and the evaporation of these substances from the surface during the drying action at super-atmospheric temperatures served to protect the surface against rapid oxidation and thus to permit the drying to proceed by the condensation reaction in the film before oxidation had dried the surface.

The reactive substances particularly desirable in the present invention may be chosen from the groups enumerated in my co-pending applications, Serial Nos. 646,148, filed December 7, 1932; 758,859; 758,860; 758,861; 758,862; 758,863; 758,864, filed December 22, 1934. Several examples are: cyclohexanol, cyclohexanone, phthalic anhydride, di-acetone alcohol, furfuraldehyde, quinone, fenchyl alcohol, fenchone, carvone, etc.

In the co-pending applications, the procedure

of improving the drying properties of drying oils having double bonds in conjugate arrangement has been described and claimed. The drying reaction is improved through the medium of a condensation reaction wherein the oil condenses with organic compounds enumerated in the various applications. Through the medium of the condensation reaction, the hardening of the film will proceed uniformly throughout the thickness of the film in contrast to the conventional hardening of oil films through oxidation. In drying films through oxidation, the surface of the film will harden first and the interior of the film tends to remain plastic. Through the medium of the hardening action of oil films, as described in the above indicated co-pending applications, in which the hardening proceeds uniformly throughout the thickness of the film, more flexible and better wearing films are acquired. It has been shown that the uniform hardening action proceeds especially in non-oxidizing atmospheres created by the slow evaporation of the volatile organic substances mixed with the oil prior to the spreading of the oil into films. If the hardening reaction is carried on in oxidizing atmospheres, the hardened film has a dull matte finish in contrast to the desirable gloss finish obtained in non-oxidizing atmospheres.

Non-reactive substances, that is, substances which will not condense with the oil when added to the drying oil, will, on being evaporated therefrom at super-atmospheric temperatures, form a protective blanket exactly as is formed in the case of the reactive substances discussed above. For example, substances such as, hydroterpene, hydrogenated naphthalene, kerosene, cymene, etc., do not condense with the drying oil when treated under circumstances described in my co-pending applications, but will, on being evaporated from the oil, form a protective blanket over the film and thereby prevent surface oxidation.

Also, generally accepted anti-oxidants which may be reactive or non-reactive with the oil such as, thymol, hydroquinone, phenol, guaiacol, resorcinol, pyrogallol, glycollic acid, furfuraldehyde, furfural, benzoic and salicylic acid,  $\alpha$ -naphthylamine, diphenylamine, phenyldimethylamine, diphenylguanidine, diphenylhydrazine, o-nitroaniline,  $\beta$ -naphthol,  $\alpha$ -terpineol, which have relatively high vapor pressures, will, on being added to the drying oil and then evaporated from the oil at super-atmospheric temperatures, form the protective blanket above the oil film as heretofore described. It is interesting to note with respect to anti-oxidants that a large percentage of oxy-compounds, classified as anti-oxidants, are reactive condensing agents with drying oils such as, China-wood oil and oils of similar structure. Similarly, as in the case of reactive substances, when a reactive anti-oxidant substance is added to the drying oil, an excess is added and the portion, which does not enter the condensation reaction with the drying oil, will form the protective blanket when evaporated from the oil. If a non-reactive anti-oxidant is added to the drying oil, the substance will form a protective gaseous blanket over the drying oil when the drying action is caused to proceed at super-atmospheric temperatures.

In cases where non-reactive substances are used in the drying oil in the absence of condensing agents, as described above, the drying of the oil proceeds by polymerization when the temperature is raised to super-atmospheric conditions and the non-reactive substance merely creates

the non-oxidizing protective blanket over the oil during the drying action.

As previously indicated, I prefer to use reactive substances, which, on being added to the oil in excess quantities, a portion will condense with the oil and the remainder will form the protective blanket as it is evaporated from the drying film. If only a sufficient quantity of reactive condensing agents is added to the drying oil to cause the condensation product to form with the oil as described in co-pending cases, a quantity of a non-reactive substance may be added to the oil to form the protective blanket. The non-reactive substance will, in this case, on being volatilized during the drying action at super-atmospheric temperatures, help to form the protective blanket.

In general, any substance which is non-oxidizing and which, when added to the drying oil in amounts up to twenty-five percent, based on the oil, will give a mixture having, between 104° F. and 212° F., vapor pressures between 2 mm. and 90 mm. column of mercury may be used. Those substances which have the lower vapor pressure ranges within the temperature range are the more desirable, and I have found, for example, that those falling within the range between 2 mm. and 60 mm. and especially those formed between 2 mm. and 50 mm. produce much better results than those extending into the higher range specified. When driers, which hasten the drying action, but ordinarily aggravate wrinkling and surface distortion, are used, it is desirable, in order to prevent or minimize wrinkling or other surface distortion, to use as protective agents those materials whose vapor pressures, within the temperature range, do not exceed approximately 25 mm.

As one example of the use of such materials according to my invention, the following may be suggested:

A vehicle may be made by hot blending the following ingredients:

|                                       | Parts by weight |
|---------------------------------------|-----------------|
| Blown China-wood oil                  | 940 45          |
| Phenol formaldehyde varnish (25 gal.) | 235             |
| Cyclohexanol                          | 115             |
| Volatile thinner                      | 155             |

The procedure of blending, which I prefer, is to place the above mixture in a Bedford kettle and blow at 200° F. or reflux at the boiling point of the mixture until it attains a desired viscosity. It is then cooled to room temperature. This forms a vehicle to which pigments and fillers may be added in the conventional manner.

When it is desired to dry the prepared mixture, the mixture is spread out in a closed chamber and heated to about 140° F. The unreacted cyclohexanol will evaporate, forming the protective film over the surface of the mixture, and the drying of the oil mixture continues until drying is complete.

As another specific example of my invention, a vehicle may be made, as follows:

38 parts by weight China-wood oil (kettle bodied to 125" viscosity) is blended with 45 parts hydroterpene and 77 parts of an ester gum varnish made, as follows:

117 parts China-wood oil  
60 parts ester gum  
150 parts petroleum thinner (safety solvent).

The varnish is hot blended with the heavy bodied China-wood oil, and the hydroterpene.

It is then cooled and the resulting vehicle may be mixed with pigments and fillers in the conventional manner. As in the previous example, the resulting mixture is spread out in a closed chamber and the temperature is raised to about 140° F. The evaporating hydroterpene will form the desired protective non-oxidizing blanket as the mixture dries to a smooth film.

In the accompanying drawings I have shown graphs of the vapor pressures of the China-wood oil mixtures within the temperature range specified for each of various protective materials.

Throughout the application, the term 7" blown China-wood oil refers to China-wood oil blown to a 7 second viscosity as determined by the Gardiner-Holt tube at 86° F.

In Figure 1 are shown for comparison graphs for 7" blown China-wood oils alone.

In Figure 2 are shown graphs of a group of materials which serve both as condensing agents and as protective agents.

In Figure 3 are shown graphs of a group of non-reactive protective agents.

On these figures the graphs represent the following materials:

A—7" blown China wood oil after heating for one hour at 95 to 97° C.

B—7" blown China wood oil untreated.

C—7" blown China wood oil and 10% indene.

D—7" blown China wood oil and 10% cyclohexanol.

E—7" blown China wood oil and 10% furfural.

F—7" blown China wood oil and 10% phenol.

G—7" blown China wood oil and 10% terpineol.

H—7" blown China wood oil and 10% butyl acetate.

I—7" blown China wood oil and 10% ethylene glycol mono butyl ether.

J—7" blown China wood oil and 10% p-menthane.

K—7" blown China wood oil and 10% kerosene.

L—7" blown China wood oil and 10% saturated naphthalene.

M—7" blown China wood oil and 10% naphthalene.

N—7" blown China wood oil and 10% phenyl ether.

O—7" blown China wood oil and 10% o-nitro toluene.

In the above I have discussed particularly the application of my invention to China wood oil. Because of the valuable properties of China wood oil which are generally recognized in the art, the greatest value of my invention at the present time will, undoubtedly, be in connection with the drying of China wood oil. It is to be understood, however, that my invention is none the less applicable to other oils which exhibit a tendency to surface distortion during drying.

The accompanying graphs disclose mixtures in which the volatile organic substances are 10% of the mixtures; however, excellent results have been obtained with mixtures in which the volatile organic substance was present in amounts up to 25% of the mixture. The disclosure of the quantity of volatile organic substance added in the examples and preceding statement shall not be construed as limiting the scope of the claims, since, if the rapidity of the hardening of the film is not of importance, the quantity of the organic substance can be varied in broad limits. If the quantity of the volatile organic substance added

to the mixture exceeds 25% of the mixture, the rapidity of the hardening action of the film is decreased.

Oils which exhibit a tendency to surface distortion during drying, but which can readily be dried with smooth and undistorted films in accord with my invention, include treated and untreated drying oils, treated semi-drying oils and non-drying oils that possess double bonds in conjugate arrangement, e. g.,  $\text{---C=C---C=C---}$  or 10  $\text{---C=C---C=C---C=}$ , (such as China wood oil, fish oils, oiticica oil, blown or properly oxidized linseed oil, blown or properly oxidized soya bean oil, blown or properly oxidized poppy-seed oil, etc., castor oil heated under reduced 15 pressures to form conjugate double bond structure and esterified, blown or properly oxidized drying oil fatty acids, and the above treated and untreated oils, having the above double bond conjugate structure, blown with drying oil fatty 20 acids or such oils to which blown or properly oxidized fatty acids have been added), fall within the scope of my invention.

As already stated, driers may be used in compositions embodying the present invention, but their use is not necessary with the highly reactive oils with which we are especially concerned, and should, in general, be avoided. Where driers are used, the difficulty of preventing wrinkling is increased, and for that reason, I have found it advantageous to use more carefully controlled drying conditions, especially as to circulation of the atmosphere, and to use the materials which in mixture with the oil show the lower vapor pressures within the range specified.

With certain of these protective materials and specifically with kerosene and with hydroterpenes, a flat or matte surface will result upon drying, whereas with others, a bright gloss will be obtained. Where a glossy surface is desired, I have found that especially good results are achieved by using a condensing agent as the slow evaporating protective agent.

Although I have set forth above in detail several specific examples and various alternatives and modifications thereof, it is to be understood that these are given only for purposes of illustration and that numerous changes which will be evident to those skilled in the art may be made without departing from the scope of my invention.

#### What I claim is:

1. In the treatment and hardening of an oxidized oil having double bonds in conjugate arrangement, the steps which comprise adding reactive volatile organic substance to the oil in excess whereby a film-forming mixture including unreacted volatile organic substance is formed, then spreading the mixture into films on a supporting base and heating the spread mixture to elevated temperatures, sufficient to simultaneously slowly evaporate the remaining volatile constituents of the film-forming mixture from the film surface forming a gaseous protective blanket over the film and substantially exclude oxidizing gases from contacting the film and sufficient to cause a substantially non-oxidizing hardening of the oil.

2. In the treatment and hardening of an oxidized oil having double bonds in conjugate arrangement, as defined in claim 1, in which the oil is China wood oil.

3. In the treatment and hardening of an oxidized oil having double bonds in conjugate arrangement, the steps which comprise adding re-

active and non-reactive volatile organic substances to the oil whereby a film-forming mixture is formed, then spreading the mixture into films on a supporting base and heating the spread mixture to elevated temperatures, sufficient to simultaneously slowly evaporate the remaining volatile constituents of the film-forming mixture from the film surface forming a gaseous protective blanket over the film and substantially exclude oxidizing gases from contacting the film and sufficient to cause a substantially non-oxidizing hardening of the oil.

4. In the treatment and hardening of an oxidized oil having double bonds in conjugate arrangement, the steps which comprise adding reactive volatile organic substance, of which a 10% mixture with said oil will give a range of vapor pressures between two and sixty mm. mercury column at temperatures between 104° and 212° F., to the oil in excess whereby a film-forming mixture including unreacted volatile organic substance is formed, then spreading the mixture into films on a supporting base and heating the spread mixture to elevated temperatures, sufficient to simultaneously slowly evaporate the remaining volatile constituents of the film-forming mixture from the film surface forming a gaseous protective blanket over the film and substantially exclude oxidizing gases from contacting the film and sufficient to cause a substantially non-oxidizing hardening of the oil.

5. In the treatment and hardening of an oxidized oil having double bonds in conjugate arrangement, the steps which comprise adding reactive volatile organic substance, of which a 10% mixture with said oil will give a range of vapor pressures between two and twenty-five mm. mercury column at temperatures between 104° and 212° F., to the oil in excess whereby a film-forming mixture including unreacted volatile organic substance is formed, then spreading the mixture into films on a supporting base and heating the spread mixture to elevated temperatures, sufficient to simultaneously slowly evaporate the remaining volatile constituents of the film-forming mixture from the film surface forming a gaseous protective blanket over the film and sub-

stantially exclude oxidizing gases from contacting the film and sufficient to cause a substantially non-oxidizing hardening of the oil.

6. In the treatment and hardening of an oxidized oil having double bonds in conjugate arrangement, the steps which comprise adding to the oil in excess of the amount necessary to react with the oil a reactive volatile organic substance in amounts up to 25 percent of the mixture, of which a 10 percent mixture with said oil will give a range of vapor pressures between two and sixty mm. mercury column at temperatures between 104° and 212° F., whereby a film-forming mixture including unreacted volatile organic substance is formed, then spreading the mixture into films on a supporting base and heating the spread mixture to elevated temperatures, sufficient to simultaneously slowly evaporate the remaining volatile constituents of the film-forming mixture from the film surface forming a gaseous protective blanket over the film and substantially exclude oxidizing gases from contacting the film and sufficient to cause a substantially non-oxidizing hardening of the oil.

7. In the treatment and hardening of an oxidized oil having double bonds in conjugate arrangement, the steps which comprise adding to the oil in excess of the amount necessary to react with the oil a reactive volatile organic substance in amounts up to 25 percent of the mixture of which a 10 percent mixture with said oil will give a range of vapor pressures between two and twenty-five mm. mercury column at temperatures between 104° and 212° F., whereby a film-forming mixture including unreacted volatile organic substance is formed, then spreading the mixture into films on a supporting base and heating the spread mixture to elevated temperatures, sufficient to simultaneously slowly evaporate the remaining volatile constituents of the film-forming mixture from the film surface forming a gaseous protective blanket over the film and substantially exclude oxidizing gases from contacting the film and sufficient to cause a substantially non-oxidizing hardening of the oil.

WALTER J. KOENIG.